

## UNITED STATES PATENT OFFICE.

GEORGES LÉPINE, OF NEUCHÂTEL, SWITZERLAND.

## UNINFLAMMABLE AND ELECTRICALLY-INSULATING LIQUID.

1,235,339.

Specification of Letters Patent.

Patented July 31, 1917.

No Drawing.

Application filed April 13, 1914. Serial No. 831,618.

*To all whom it may concern:*

Be it known that I, GEORGES LÉPINE, a citizen of the Republic of France, residing at Neuchâtel, Canton of Neuchâtel, in the 5 Confederation of Switzerland, have invented certain new and useful Improvements in Uninflammable and Electrically-Insulating Liquids, of which the following is a specification.

10 It has been already proposed to render partially uninflammable the oil which usually is employed as insulating material in electrical apparatus such as oil break switches, transformers and the like, by mixing it with uninflammable substances. Thereby a liquid is obtained which at ordinary temperature and up to 100° Celsius is not inflammable, but once heated to a higher temperature becomes again inflammable because the uninflammable substance which has been added to the oil has evaporated.

15 The subject of the present invention consists in a liquid which contrarily to the above mentioned mixture is uninflammable in all its parts and forms an excellent substitute for the inflammable oil usually employed in the electrical apparatus.

20 The liquid according to the present invention consists of at least one chlorin compound of hydrocarbons such as the olefins and the hydrocarbons of the benzene series or others. It may consist for instance of pentachlorethane ( $C_2HCl_5$ ) alone or mixed with one or more chlorin compounds of the olefins such as for instance dichlorethane (Dutch liquid)  $C_2H_4Cl_2$ , hexachlorethane  $C_2Cl_6$ , or of the hydrocarbons of the benzene series such as for example trichlorobenzene  $C_6H_3Cl_3$ , tetrachlorobenzene  $C_6H_2Cl_4$ , pentachlorobenzene  $C_6HCl_5$  and hexachlorobenzene  $C_6Cl_6$ .

25 The liquid may also consist of pentachloropropane, tetrachloropropane and hexachloropropane and contain a substance capable of fixing the products of eventual decomposition, which would be noxious to the metals. This substance may advantageously consist of toluidin.

30 The uninflammable liquid may also consist of a mixture of pentachlorethane with a compound obtained by passing chlorin, while heated, into certain petroleum-oils containing unsaturated hydrocarbons.

35 The composition of the liquid may vary. Some examples of its composition will now be described.

*Example I.*

93 per cent. pentachlorethane (boiling point 160° C.)  
 5 " " dichlorethane (Dutch liquid) (84° C.)  
 2 " " hexachlorethane (boiling point 185° C.)

This mixture is made by first dissolving the hexachlorethane in the pentachlorethane, and by mixing the obtained solution with the dichlorethane. Thereby a viscous liquid is obtained which has the property of giving off vapors when it is heated at about 80° C. The characteristic odor of the vapors produced have the advantage of indicating for instance, a probable perturbation of an electric apparatus (break switch) in which the liquid is employed as a substitute for the oil which is usually employed.

45 This liquid when gradually heated in an open crucible, until vapors evolve, does not take fire even when a coal-gas flame is directed into the vapors, but the vapors extinguish the flame.

50 Essays have been made for determining the dielectric properties of the liquid having the above named composition. These essays gave the following results:

55 The electric puncture test has been made between two points which were immersed in the liquid the temperature of which was 17° C. The sparking distance was 10 millimeters and the tension was gradually increased until the first spark occurred. The tension was furnished by a transformer of 20 kilowatts at 100000 volts at 50 cycles per second. The first spark took place at 30000 65 90 volts.

60 The liquid was then submitted to another test relating to the decomposition by electric spark. About 20 sparks per minute were passed through the liquid for 20 minutes. 95 The liquid became black and opaque and its temperature was nearly that of the hand. After cooling to ordinary temperature of about 17° C. the liquid was again submitted to a puncture test under the same conditions 100 as before and the first spark took place at 21400 volts.

65 The insulation resistance measured at a tension of 1000 volts and at a temperature of 16° C. is 726 megohms per cubic-centimeter.

*Example II.*

70 80 per cent. pentachlorethane.  
 18 " " pentachlorobenzene.  
 2 " " hexachlorobenzene with the addition of  
 1 " " toluidin.

75 This mixture is made as follows:  
 The pentachlorobenzene and the hexachlo-

65

70

75

80

85

90

95

100

105

110

robenzene are dissolved in the pentachlor-  
ethane and 1 per cent. toluidin is added in  
order to fix the bodies which owing to de-  
composition would be injurious to metals  
5 and would then become electric conductors,  
owing to the said decomposition.

This liquid heated in an open crucible be-  
haves like the liquid described in the first  
example. It does not take fire and the escap-  
10 ing vapors extinguish a coal-gas flame  
directed into them.

The electric puncture test has been made  
between two points immersed in the liquid  
at 18° C. The spark distance between the  
15 two points varied from 2.5 to 10 mm. and  
the tension was gradually raised until the  
first spark occurred. The tension was sup-  
plied by a transformer of 20 K.W. of 100000  
20 volts at 50 cycles per second like in the first  
example.

The following are some values of tensions  
at which the first spark occurred:

| 25        | Spark distance mm. | Minimal<br>volts. | Maximal<br>volts. | Mean of 6<br>punctures. |
|-----------|--------------------|-------------------|-------------------|-------------------------|
| 2.5.....  | 11,600             | 16,100            | 13,650            |                         |
| 5.0.....  | 22,000             | 22,500            | 22,300            |                         |
| 10.0..... | 36,900             | 44,600            | 41,000            |                         |

30 The insulating resistance is identical to  
that of the liquid described in the first ex-  
ample.

*Example III.*

35 The pentachlorethane may also be mixed

with a compound obtained by passing chlo-  
rin, while heated, into certain petroleum  
oils containing unsaturated hydrocarbons.  
This compound must however be distilled  
before being mixed with the pentachlor-  
40 ethane, in order to remove any hydrocarbon  
which would not have been transformed into  
a chlorinated compound.

By this mixture a viscous liquid is ob-  
tained, which is completely incombustible 45  
and is a good electrical insulator. The boil-  
ing point of this liquid varies between 160°  
and 326° C.

I claim as my invention:

1. An uninflammable and insulating liq-  
uid 50 comprising a mixture of pentachlore-  
thane and a chlorin compound of the elefins.

2. An uninflammable and insulating liquid  
comprising a mixture of pentachlorethane  
and dichlorethane.

3. An uninflammable and insulating liquid  
comprising a mixture of pentachlorethane,  
dichlorethane and hexachlorethane.

4. An uninflammable and insulating liquid  
comprising a mixture of 93 per cent. penta-  
55 chlorethane, 5 per cent. dichlorethane and 2  
per cent. hexachlorethane.

In testimony whereof I have affixed my  
signature in presence of two witnesses.

GEORGES LÉPINE.

Witnesses:

D. ROD. DE WURTEMBERG,  
LOUIS H. MUMOR.